

## UNITED STATES PATENT OFFICE

2,578,356

PROCESS OF REMOVING BACKS FROM  
MARINE AND FRESH WATER SHELLSJoseph H. Hooton, Englewood, N. J., assignor to  
Richelieu Corporation, New York, N. Y., a corporation of New YorkNo Drawing. Application March 24, 1949,  
Serial No. 83,289

3 Claims. (Cl. 252—1)

1

This invention relates to a novel process of removing backs from marine and fresh water shells.

Many marine and fresh water shells consist largely of a very attractive mother-of-pearl or nacre. This mother-of-pearl or nacre is made up of laminations of flat calcium carbonate particles (sometimes called, crystals, scales, or platelets) held together by a proteinaceous substance known as conchiolin. Such shells are very attractive on the inside thereof but the outside surface is rough, scaly, porous, dull and very unattractive. Very attractive objects are sometimes made by grinding off the outside surface and polishing the area underneath the surface. The grinding process, however, is a difficult and laborious process. If it is desired to obtain the lamellar crystals or nacreous material from the shells it is also desirable to remove the back portion to prevent contamination of the crystal products.

It has already been proposed to exfoliate the lamellae, or laminae of such shell by heat treating in an oven (see U. S. Patent No. 1,570,183), by heating with water under pressure (see U. S. Patent No. 1,812,885) or by treating with a mild alkaline solution with or without extraneous heating (see U. S. Patent 2,172,369). Such treatments appear to soften the proteinaceous binding material holding the laminae together so that the particles are easily separated. None of the above mentioned patents refer to any method of removing the backs from shells but it is presumed that either the backs are first removed by grinding or that the contaminating material of the back of the shell which cannot be removed by subsequent washing or decanting is permitted to remain in the product.

The normal method of removing the backs of such shells is by grinding with high speed abrading wheels. This process is expensive, laborious and creates a considerable amount of harmful and annoying dust.

An object of this invention is to provide a novel method of removing the backs of such marine or fresh water shells without exfoliating or otherwise disturbing the remainder or nacre-containing portion of the shell.

Another object of the invention is to provide a chemical method of removing the backs of marine and fresh water shells without exfoliating or otherwise destroying the nacre of the shell.

These results and others ancillary thereto are obtained by treating the shells at low pressure and relatively low temperatures in an autoclave with an aqueous solution. The treatment is such

2

that, if higher temperature or a longer time of treatment were employed, exfoliation might result. It has been found, however, that the backs can be removed by a considerably milder type of treatment than that required for exfoliation. This may be due to the porous nature of the backs or it may be due to some other chemical or physical factor.

The exact temperature and pressure limits cannot be precisely defined since there is a wide range of such limits. The pressure which is employed is the pressure which corresponds to the vapor pressure of the water vapor in the treating solution at the required temperature. As a practical matter temperatures of 102° C. to 198° C. (corresponding to steam gauge pressures of about 1 to 200 p. s. i.) may be employed. The time element, however, is important in that the process is stopped before any exfoliation of the interior of the shell takes place. The lower the temperature and pressure the longer it is necessary to treat the shells. Under the treatment as usually conducted, cracks appear in the back of the shells and the large fragments defined by the cracks separate at the edges from the rest of the shell and can be easily removed by hand or by passing under a brushing mechanism.

The aqueous solution which is employed can be ordinary tap water if the temperature is raised sufficiently but preferably the water is made slightly alkaline. The best alkaline agent for effecting the separation of the back, at such a rate that there is no exfoliation of the remainder of the shell, are the alkali phosphates such as trisodium phosphate, disodium phosphate and mixtures thereof.

The novel features characteristic of this invention are set forth with particularity in the appended claims. The invention itself, however, both as to its organization and its method of operation, together with additional objects and advantages thereof, will best be understood from the following description of specific embodiments when read in connection with the accompanying examples in which:

## Example 1

A solution of seven pounds of trisodium phosphate in six gallons of water is poured over red or green abalone shells which have been placed in an autoclave so that all of the shells are submerged in the water. The temperature is then raised to about 174° C. (corresponding to about 111 p. s. i. steam gauge pressure). The process is continued for about two hours when the steam

pressure is turned off and the shells are permitted to remain in the autoclave until cooled.

When the shells are removed from the autoclave it is found that the back breaks off in large fragments when subjected to shearing stress.

*Example 2*

A quantity of shells having the scientific name of *Placuna Sella Gmelin* is placed in an autoclave so as to substantially half fill the same. Sufficient trisodium phosphate solution containing about a pound of commercial trisodium phosphate per gallon of water is added to completely submerge the shells. The autoclave is then closed and the shells are treated at about 178° C. (corresponding to about 125 p. s. i. of steam gauge pressure) for 100 minutes.

The loosened backs can be easily removed by brushing with a wire brush.

I claim:

1. A process of removing backs from marine and fresh water shells comprising the steps of placing the shells in an autoclave, covering said shells with an aqueous solution of an alkali phosphate selected from the group consisting of the trialkali phosphates and the dialkali phosphates and mixtures thereof, closing the autoclave, subjecting the shells to heat treatment corresponding to steam gauge pressure of 1 to 200 p. s. i. for a sufficient time to cause the backs of the shells to crack and separate from the remainder of the shell, and then stopping the treatment before any exfoliation of the body of the shells takes place.

2. A process of removing backs from marine

35

and fresh water shells comprising the steps of subjecting the shells to heat treatment corresponding to steam gauge pressure of 1 to 200 p. s. i. in the presence of an aqueous solution of trisodium phosphate, for a sufficient time to cause the backs of the shells to crack and separate from the remainder of the shell, and then stopping the treatment before any exfoliation of the body of the shells takes place.

10 3. A process of removing backs from marine and fresh water shells comprising the steps of subjecting the shells to heat treatment corresponding to steam gauge pressure of 1 to 200 p. s. i. in the presence of an aqueous solution of trisodium phosphate for a sufficient time to cause the backs of the shells to crack and separate from the remainder of the shell, stopping the treatment before any exfoliation of the body of the shells takes place, removing the shells from the 15 autoclave and separating the shell backs from the body of the shell by applying shearing stress to the backs of the shells.

JOSEPH H. HOOTON.

REFERENCES CITED

The following references are of record in the file of this patent:

UNITED STATES PATENTS

| 30 | Number    | Name         | Date           |
|----|-----------|--------------|----------------|
|    | 1,570,183 | Rouschenberg | Jan. 19, 1926  |
|    | 1,812,885 | Lippincott   | July 7, 1931   |
|    | 1,823,136 | Frederick    | Sept. 15, 1931 |
|    | 2,306,292 | Atwood       | Dec. 22, 1942  |
|    | 2,380,741 | Fischer      | July 31, 1945  |